

Aug. 26, 1952

W. L. FINLAY ET AL

2,608,140

SHOT SHELL MANUFACTURE

Filed Feb. 15, 1947



Fig. 1



Fig. 2

INVENTORS  
WALTER L. FINLAY  
BY DOROTHY R. ADESSA  
*Signature*  
John H. Lewis Jr. ATTORNEY

## UNITED STATES PATENT OFFICE

2,608,140

## SHOT SHELL MANUFACTURE

Walter L. Finlay, Fairfield, and Dorothy R. Adessa, Bridgeport, Conn., assignors to Remington Arms Company, Inc., Bridgeport, Conn., a corporation of Delaware

Application February 15, 1947, Serial No. 728,790

2 Claims. (Cl. 93—83)

1

This invention relates to ammunition, particularly to shot shells, and contemplates a novel method of manufacture which enables the use of lower cost materials.

The conventional shot shell as used extensively for small game hunting and skeet and trap shooting comprises a primer, base wall, powder charge, filler walls, and shot charge; all housed in a container which ordinarily consists of a metallic cup-shaped head and a tubular body. While the body may be of metal and may be integral with the head, in common practice the body is of a non-metallic material, and while the use of various plastics has been attempted the body is almost universally formed of a rolled sheet of paper. In the firing of such a shot shell in the gun chamber, the shell is subjected to an interior pressure of the order of 10,000 pounds per square inch and inevitably expands until it is supported by the chamber wall. By reason of the fact that commercial shot shells are used under an extremely wide variety of conditions of temperature and atmospheric humidity, an allowance must be made for the swelling of the non-metallic body by the absorption of moisture. Accordingly, shot shells are finished to an outside diameter which is somewhat less than the minimum average chamber diameter of a new gun and substantially less than the chamber diameter of an old and worn gun. When the shell is fired, the body material must stretch without longitudinal rupture until it is engaged by the chamber wall. It is essential that such body splits be avoided, since a body split may expose the breech mechanism to a flow of burning gas under high pressure, with damage to the gun action and possible injury to the shooter.

Throughout the history of the manufacture of paper bodied shot shells, it has been deemed necessary to use a paper especially manufactured to provide a very high transverse stretch or elongation to permit the necessary transverse enlargement of the shell body on firing. Ordinary paper does not possess this property. Shot shell paper is quite universally made by superposing four plies of a thin web produced on a "cylinder" machine. A specially prepared and extensively beaten pulp stock is introduced into a tank containing a horizontally disposed revolving screen cylinder. The water level within the cylinder is maintained several inches below the stock level outside the cylinder. As the screen cylinder revolves, the water of the pulp stock passes through the screen and pulp fibers adhere to its surface. The web thus formed is

2

removed from the cylinder by contact with a moving felt blanket. Special devices to provide a uni-directional flow of pulp stock toward the cylinder are provided, the whole combination resulting in a web in which a substantial portion of the fibers are laid lengthwise. By building a sheet of four such webs, a transverse stretch or elongation up to 12% or 15% is secured. The absolute minimum requirement for paper to be processed into shot shells by heretofore known methods is a transverse elongation of 9%. It is quite obvious that this cylinder process is much more expensive than the "Fourdrinier" process, in which the stock is simply flowed from the tank in a flat stream onto a longitudinally moving and vibrating screen, from which a full sheet thickness web is continuously removed. While in this process there is still considerable lengthwise laying of fiber, there is a substantially greater random orientation, and while transverse elongation is somewhat greater than longitudinal elongation, the former rarely exceeds 6%. Such paper has heretofore been deemed wholly unsuitable for the manufacture of shot shells.

The present invention contemplates a process which enables the utilization of relatively low cost Fourdrinier paper, instead of high cost specially made composite sheet cylinder paper. The utility of the process, however, is not limited to Fourdrinier paper; its application to the specialty papers customarily used, and variations of such papers, results in a marked improvement in quality.

35 In the drawings:

Fig. 1 is a diagrammatic representation of end views of shot shell tubes made in accordance with the present invention, illustrating the relative diameters of the tube as wound, the tube as sized, and the shot shell body after firing.

40 Fig. 2 is a fragmentary diagrammatic sectional view of the tube sizing devices.

45 There are several factors which effect the fit and behavior of a shot shell in different guns. Gun chambers are contracted forwardly from the breech end or "mouth" toward the "forcing cone," the taper of a new chamber being about .005" per inch. A certain variation or "tolerance" necessarily exists in the dimensions of new gun chambers, and with extensive use an indefinite amount of chamber enlargement takes place. A certain tolerance is likewise necessary in shell diameter. Again, the shell wall may be thicker in some parts than in others. The usual 50 convolute 12 gauge tube, for example, comprises

about four-and-one-half turns of paper, and is thus 20% thicker on one side than on the other; this produces an asymmetric stress pattern. The load applied upon firing is an impact load, and the effect differs from that of a static load.

"Average" chamber diameter as used herein indicates mean diameter of a new chamber midway of its length. As mentioned above, shot shell bodies must be finished to an outside diameter somewhat less than the average minimum chamber diameter. Prior to the present invention, it has been the universal practice to make shot shell tubes by winding paper sheets upon an arbor of such dimensions that the outside diameter of the tube as wound does not exceed average chamber diameter. Such tubes, after drying, were then sized to the required exterior diameter by being impaled upon a mandrel and pushed through a sizing die. Upon firing in an average chamber, the sized tube should theoretically be symmetrically stressed and expand to its wound diameter, but, due to the asymmetry of the tube itself, the impact load, and probably other factors, the stressing of the tube, even in a new chamber, is irregular and localized. When fired in a loose or worn chamber, any or all of these stress effects tend to be intensified, with the result that the use of paper having a high transverse elongation has heretofore been deemed a necessity. The present invention comprises the discovery of a process which enables the use of ordinary Fourdrinier paper having a transverse elongation far less than that heretofore considered necessary.

Fourdrinier paper of a thickness substantially equal to that of standard specialty shot shell paper is wound on an oversize mandrel, the outside diameter of the wound tube being substantially greater than average chamber diameter as above defined. The cross-section of such a tube is shown at the left in Fig. 1. At the right in Fig. 1 is a diagrammatic showing of a section of a gun chamber of an average diameter  $d$ , and the measure of this diameter is extended across the figure for the purpose of comparison. It will be noted that the tube as wound (shown at left in Fig. 1) is of considerably greater diameter than the gun chamber.

The oversize wound tube is next humidified to such a moisture content as will enable severe sizing, that is, sizing down to the usual outside diameter, shown in the center of Fig. 1. If the tube contains inadequate moisture, it may be sized down to the required exterior diameter but may not retain this diameter in storage. For ordinary Fourdrinier kraft paper, minimum practicable moisture content at sizing is of the order of 10%. The maximum permissible moisture content depends upon the character of the sizing equipment. Over-humidified tubes are soft and require special handling. With conventional sizing equipment, the maximum permissible moisture content is of the order of 18%. Standard specialty shot shell paper may be sized according to the present invention with a moisture content substantially less than that required for Fourdrinier kraft, say 7%, or even less. In general, the moisture content necessary for proper sizing depends upon the degrees of hydration (beating) and/or bleaching of the stock from which the paper is laid.

The humidified tubes are next sized with substantially conventional tools to standard outside dimensions. A section of the sized tube is shown in the middle of Fig. 1 and it will be noted that

its diameter is substantially less than the diameter of the unsized tube shown at the left and is less than the average chamber diameter  $d$  by the usual amount. Fig. 2 shows, somewhat schematically, the sizing equipment. The oversize tube  $T$  is impaled on a mandrel  $10$  of conventional design. A part or all of the mandrel surface may be roughened or corrugated as shown at  $11$ , in accordance with common practice. The end of the tube abuts a thrust collar  $12$  secured to the mandrel. The mandrel reciprocates with respect to a stationary sizing die  $13$  of conventional construction. Due to the fact that the tube is oversize, it fits loosely upon the standard size mandrel  $10$  but, as the leading end of the tube and mandrel enter the throat of the die, the end portion of the tube is compressed into gripping engagement with the mandrel and the remainder of the tube is virtually pulled through the die by frictional engagement of the sized portion of the tube with the mandrel.

The sized tubes are thereafter processed in the usual manner and assembled with the other components of a shot shell. Many thousands of shot shells have been made in this manner from different lots of Fourdrinier kraft paper having a transverse elongation not over 6%. These shells were subjected to the usual severe acceptance tests and found to be in all respects equal, if not superior, to shot shells made by conventional methods from expensive specialty paper.

The invention may be illustrated by this example: Tubes for 12 gauge shot shells were wound to outside diameters as follows:

Maximum .835 Minimum .825 Average .830

After appropriate humidification, these tubes were sized to outside diameters:

Maximum .787 Minimum .781 Average .784

The maximum diameter reduction is approximately 6.5%; the minimum reduction is approximately 4.6%; and the average reduction is 5.5%. The maximum diameter reduction in conventional processing, under the more liberal tolerances provided for commercial manufacture, does not exceed about 2.6%, and probably only rarely approaches this figure.

The severe sizing enables the use of many lower grade papers. No transverse elongation minimum has been found. Satisfactory shooting results have been secured with Fourdrinier kraft having a transverse elongation as low as 1.6%.

The invention is not limited to tubes of any particular size or style of winding. It is applicable to tubes of any size, and to spiral or parallel wound tubes as well as to the more common convolute tubes.

What is claimed is:

1. In the manufacture of tubes for shot shell bodies from Fourdrinier kraft paper, the method which comprises winding and adhesively securing paper into tubes of a diameter not less than 5% greater than the desired finished diameter, humidifying such wound tubes to a moisture content determined by the transverse elongation of the paper but not less than 7% or more than 18%, and compressing the humidified tubes to reduce the diameter by not less than 4.5%.

2. In the manufacture of bodies for shot shells for use in gun chambers of varying average diameter, the method which comprises winding and adhesively securing paper having a transverse elongation not substantially exceeding 6% into tubes having an outside diameter not materially

less than 5% greater than maximum average chamber diameter, humidifying such wound tubes to a moisture content between 10% and 18%, the moisture content being determined by the transverse elongation of the paper, and thereafter reducing the outside diameter of the wound tubes to less than minimum average chamber diameter.

WALTER L. FINLAY.  
DOROTHY R. ADESSA.

## REFERENCES CITED

The following references are of record in the file of this patent:

## UNITED STATES PATENTS

| Number    | Name     | Date          |
|-----------|----------|---------------|
| 887,809   | Hurd     | May 19, 1908  |
| 1,412,018 | Keller   | Apr. 4, 1922  |
| 1,623,965 | Marshall | Apr. 12, 1927 |
| 1,959,109 | Rosien   | May 15, 1934  |
| 2,034,731 | Saalbach | Mar. 24, 1936 |
| 2,266,420 | Gardner  | Dec. 16, 1941 |

## OTHER REFERENCES

Chemical Engineering Handbook—page 1088,  
2nd Ed., McGraw-Hill Pub. Co., 2nd Ed., 1941.